

S. M. BULLOCK AND H. S. LLOYD.  
ABRASIVE DISK WHEEL.  
APPLICATION FILED JULY 15, 1919.

1,351,021.

Patented Aug. 31, 1920.

Fig. 1



Fig. 2



Witnesses

Wm. M. Jackson  
Charles H. Lloyd

Inventors

Samuel M. Bullock  
Harry S. Lloyd  
D. C. Watt

# UNITED STATES PATENT OFFICE.

SAMUEL M. BULLOCK, OF CHICAGO, AND HARRY S. LLOYD, OF OAK PARK, ILLINOIS.

## ABRASIVE-DISK WHEEL.

1,351,021.

Specification of Letters Patent. Patented Aug. 31, 1920.

Application filed July 15, 1919. Serial No. 310,968.

To all whom it may concern:

Be it known that we, SAMUEL M. BULLOCK and HARRY S. LLOYD, citizens of the United States, and residents of the city of Chicago and village of Oak Park, respectively, in the county of Cook and State of Illinois, have invented certain new and useful Improvements in Abrasive-Disk Wheels; and we do hereby declare that the following is a full, clear, and exact description of the same, reference being had to the accompanying drawings, and to the numerals of reference marked thereon, which form a part of this specification.

15 This invention relates to abrasive disks, more particularly those used in disk grinders in which the face of the wheel is employed for grinding purposes of our Patent No. 1,311,550, issued July 29th, 1919.

20 The problem of constructing satisfactory abrasive disks is a difficult one and various attempts have been made to solve it with only partial success.

Abrasive disks must be made relatively 25 very thin to avoid the disk breaking under the action of centrifugal force and also to avoid the necessity of supporting the axle which carries the disk on each side of the grinding surface.

30 When glue is employed as a binder the practical limit of thickness is about  $\frac{3}{2}$ " but disks made by our improved method may be considerably thicker. Thus an 18" disk made by our process may be  $\frac{3}{16}$ " thick and a 53" disk  $\frac{3}{8}$ " thick. Usually the thickness of the disks is less than  $1\frac{1}{2}$ % and more rarely between  $1\frac{1}{2}$  and 5% of their diameter.

It is impractical to make such disks by baking owing to the shrinkage and distortion produced by the heat, especially in a disk as thin as above specified.

If glue is employed as the binder the disks must be made excessively thin since as soon as the surface layer of adhesive has worn off and the glue binder is exposed the heat produced by the friction of the disk against the surface being ground causes the glue to melt and flow over the surfaces of the abrasive particles and thereby inhibits their cutting action.

By using a binder composed of magnesium chlorid and magnesium oxid a grinding disk can be made which will retain its

cutting action until it has been worn completely away.

Difficulty has, however, been experienced in mounting disks of this character owing to the trouble involved in cementing the disk to its support. We have found that this difficulty may be overcome by using a 55 fabric base for the disk. The fibrous nature of the fabric provides an excellent bonding medium between the abrasive and magnesium mixture on the one hand and also provides a satisfactory support for the glue by 60 which the disk so formed may be secured to the metallic surface of a driving wheel.

It has further been found that if the wet mixture of abrasive, magnesium chlorid and magnesite is applied to a dry fabric disk 70 the latter absorbs the magnesium chlorid solution from the mixture and seriously interferes with the setting so that instead of a rock-like surface a soft friable surface is obtained.

This difficulty may be overcome by wetting the fabric before applying the abrasive mixture thereto either with plain water or preferably with a strong solution of magnesium chlorid.

It is an object, therefore, of this invention to provide an improved grinding disk which will retain its cutting qualities to the last and which may be readily and securely attached to a driving wheel.

Other and further important objects of this invention will be apparent from the disclosures in the specification and drawings.

The invention (in a preferred form) is illustrated in the drawings and hereinafter 90 more fully described.

### On the drawings:

Figure 1 is a front elevation of a disk and driving wheel embodying the features of the present invention.

Fig. 2 is a section on the line 2—2 of Fig. 1.

### As shown on the drawings:

The fabric disk 2 is first wetted, preferably with a strong solution of magnesium chlorid. Then a mixture of abrasive particles, magnesite and magnesium chlorid is applied to the disk to form a layer 1 of the desired thickness. The whole then sets in the course of a few hours to a hard rock-like disk by reason of the peculiar proper-

ties of magnesium chlorid and its power to combine with magnesite to form a hard substantially insoluble oxychlorid.

The abrasive mixture may conveniently be made in the following proportions:

5 75% of a suitable abrasive such as carborundum,

12½% of magnesium chlorid,

12½% of calcined magnesite.

10 Sufficient water is employed to bring the magnesium chlorid into solution.

For wetting the fabric disk a solution of magnesium chlorid containing about 85% by weight of the salt may be used.

15 In applying the abrasive mixture to the fabric disk any convenient method may be employed such as pressing, tamping, pounding or rolling either by hand or machine.

After the disk has set it may be secured 20 to a driving wheel 3 by applying any suitable adhesive such as sodium silicate or water glass to the surface of the fabric 2 and, after clamping the disk against the wheel, allowing the same to dry. This will 25 serve to hold the disk rigidly associated with the driving wheel until the disk has become worn necessitating removal thereof. The

fabric and remaining portion of abrasive may be torn from the wheel or the glue or cement may be dissolved by any suitable solvent to permit easy removal of the fabric and the remainder of the abrasive thereon.

We are aware that numerous details of construction may be varied through a wide range without departing from the principles 35 of this invention, and we therefore do not purpose limiting the patent granted otherwise than necessitated by the prior art.

We claim as our invention:

An abrasive disk for disk grinders comprising a fabric disk and a layer of abrasive particles bound together and to the fabric by magnesium chlorid and magnesite, the ratio of magnesium chlorid to magnesite being higher in the fabric than in the layer 45 of abrasive material.

In testimony whereof we have hereunto subscribed our names in the presence of two subscribing witnesses.

SAMUEL M. BULLOCK.  
HARRY S. LLOYD.

Witnesses:

EARL M. HARDINE,  
CHARLES W. HILLS, Jr.